

# United States Patent Office

2,795,479

Patented June 11, 1957

1

2,795,479

## METHOD FOR CONVERTING URANIUM AMMONIUM PHOSPHATE TO URANYL FLUORIDE

Seymour Bernstein and Harvey A. Bernhardt, Oak Ridge, Tenn., assignors to the United States of America as represented by the United States Atomic Energy Commission

No Drawing. Application April 25, 1950,  
Serial No. 158,062

10 Claims. (Cl. 23—14.5)

Our invention relates to a method of converting uranyl ammonium phosphate to other uranium values and more particularly to the conversion of uranyl ammonium phosphate to  $\text{UO}_2\text{F}_2$ .

It has been discovered that it is advantageous to recover uranium from certain waste solutions in the form of various uranyl phosphate precipitates, such as uranyl hydrogen phosphate, uranyl sodium phosphate, and particularly uranyl ammonium phosphate. However, it has been found extremely difficult to treat these precipitates in order to economically convert the uranium contained therein into a form, such as  $\text{UF}_6$ , which is readily returnable to various plant processes. Attempts to fluorinate these uranyl phosphates directly to  $\text{UF}_6$  have resulted in the formation of by-product phosphorous fluorides which consume costly elemental fluorine and are difficult to separate from the  $\text{UF}_6$ . Efforts have therefore been made to produce  $\text{UO}_2\text{F}_2$  as an intermediate compound since it is known that  $\text{UO}_2\text{F}_2$  may be feasibly converted to  $\text{UF}_6$  by reaction with fluorine. Hydrofluorination of uranyl ammonium phosphate, however, proved unsatisfactory for a commercial process since it resulted in the formation of the corrosive by-product ammonium hydrogen fluoride ( $\text{NH}_4\text{HF}$ ) which is a solid at room temperature and which plugs process exhaust lines and valves.

An object of our present invention, therefore, is to provide a process for converting uranyl ammonium phosphate into another uranium compound which is easily and economically convertible to  $\text{UF}_6$ .

Another object of our invention is to provide an improved method for converting uranyl ammonium phosphate to  $\text{UO}_2\text{F}_2$ .

A further object is to provide a process for substantially quantitatively converting uranyl ammonium phosphate to  $\text{UO}_2\text{F}_2$  without the formation of corrosive by-products which are solids at room temperature.

Additional objects and advantages of our invention will be apparent from the following description.

In accordance with our present invention, the substantially complete conversion of uranyl ammonium phosphate to  $\text{UO}_2\text{F}_2$  may be effected in an economically feasible manner by heating the uranyl ammonium phosphate within a narrow temperature range until substantially all the uranyl ammonium phosphate is converted to uranyl hydrogen phosphate, and then contacting the resulting uranyl hydrogen phosphate with anhydrous HF at a suitably elevated temperature until substantially all the uranyl hydrogen phosphate is converted to  $\text{UO}_2\text{F}_2$ .

Using this two step method, we avoid the formation of the extremely undesirable  $\text{NH}_4\text{F}\cdot\text{HF}$  mentioned above and also obtain a product which is very reactive with many reagents but which we find is particularly suitable for reaction with fluorine to form  $\text{UF}_6$  without the expenditure of the economically unfeasible amount of fluorine which would be required to directly fluorinate any of the uranyl phosphates described above.

In general, any form of uranyl ammonium phosphate may be effectively decomposed in the preliminary step

2

of our process to form uranyl hydrogen phosphate. However, the uranyl ammonium phosphate which is commonly recovered from waste solutions is



and we have discovered that unexpected advantages result from drying this  $\text{UO}_2\text{NH}_4\text{PO}_4\cdot 4\text{H}_2\text{O}$  to



10 and utilizing the latter for decomposition to uranyl hydrogen phosphate. We find that this drying may be easily accomplished, for example, by heating the



15 at a temperature of approximately 50° C. to approximately 80° C. for approximately 6 hours to approximately 24 hours at atmospheric pressure. However, a temperature of about 60° C. is generally preferred.

The resulting  $\text{UO}_2\text{NH}_4\text{PO}_4\cdot 2\text{H}_2\text{O}$  is much easier to handle than the original  $\text{UO}_2\text{NH}_4\text{PO}_4\cdot 4\text{H}_2\text{O}$  and there is a marked improvement in the absence of  $\text{NH}_3$  from the uranyl hydrogen phosphate product of the following decomposition step.

The temperature for the conversion of uranyl ammonium phosphate to uranyl hydrogen phosphate is 25 somewhat critical, for a greatly increased rate of formation of uranyl hydrogen phosphate appears to fall within the region of approximately 450° C. Uranium phosphate compounds other than uranyl hydrogen phosphate tend to be formed in progressively larger amounts as the temperature is increased above 450° C., for the same reaction period. During the following hydrofluorination step, these phosphates would form uranium compounds other than the desired  $\text{UO}_2\text{F}_2$ . At temperatures substantially lower than 450° C., the decomposition reaction becomes 30 uneconomically slow. The decomposition should therefore be effected within the range of 300° C.—500° C., and preferably at approximately 450° C.

We find that the time of the decomposition reaction is 35 important in obtaining a high purity product uranyl hydrogen phosphate. Although a two hour period provides satisfactory results, and complete removal of  $\text{NH}_3$ , a period of four to five hours appears to be best.

During the decomposition reaction, it is desirable to 40 sweep out gaseous decomposition products by means of an inert gas. Although, in general, any inert gas may be used for this purpose, air has been found to be completely satisfactory and is obviously to be preferred for 45 reasons of economy. The quantity of gas flow is not critical but insufficient flow retards the decomposition 50 reaction. In general, we find that a gas velocity of approximately 2.7 cm./sec. to approximately 4.1 cm./sec. per 10 grams of starting material removes the decomposition products approximately as fast as they are formed when the reaction conditions described above are utilized.

55 In the final step of our invention, the temperature for the hydrofluorination of uranyl hydrogen phosphate to  $\text{UO}_2\text{F}_2$  is not as critical as the temperature for the preceding decomposition step. However, we find that a range of approximately 400° C. to approximately 500° C. is 60 particularly advantageous, and the optimum temperature appears to be about 500° C.

An anhydrous HF gas velocity of approximately 0.82 cm./sec. to approximately 1.1 cm./sec. per 10 grams of uranyl hydrogen phosphate effects substantially complete 65 conversion to  $\text{UO}_2\text{F}_2$  in an optimum time, although the higher part of this range appears to cause the reaction to proceed somewhat faster without deleterious side effects.

The time of the reaction is not critical but depends upon 70 the particular combination of quantities and reaction conditions described above. For example, if a gas velocity of 1.1 cm./sec. of anhydrous HF per 10 grams uranyl hydrogen phosphate is utilized at a temperature of about

500° C., approximately 3 hours appear to provide optimum results. If a gas velocity of 0.82 cm./sec. is utilized, approximately 4 hours appear to be best.

In a preferred procedure for carrying out the two step conversion of uranyl ammonium phosphate to  $\text{UO}_2\text{F}_2$  in accordance with our invention,  $\text{UO}_2\text{NH}_4\text{PO}_4\cdot 2\text{H}_2\text{O}$  is placed in HF resistant reaction trays in an HF resistant reactor, which is then inserted in a furnace. The air flow is started through the reactor, as the furnace is turned on, at a velocity of approximately 4.1 cm./sec. per 10 grams starting material. The reaction zone is heated to a temperature of about 450° C. and maintained there for approximately four hours. The air flow is then cut off, the temperature raised to approximately 500° C., and anhydrous HF gas, at a velocity of approximately 0.82 cm./sec. per 10 grams starting material, is passed through the reaction zone for about four hours. The material remaining in the reaction trays is the  $\text{UO}_2\text{F}_2$  product.

After treating uranyl ammonium phosphate in accordance with the above procedure, we find that the  $\text{UO}_2\text{F}_2$  product is approximately ninety-eight percent pure and may be readily and economically fluorinated to form  $\text{UF}_6$  of sufficient purity for practically any desired use.

The following specific example illustrates our invention in greater detail.

*Example I*

A charge of 11 grams of  $\text{UO}_2\text{NH}_4\text{PO}_4\cdot 4\text{H}_2\text{O}$  was dried at 60° C. for 16 hours. The resulting  $\text{UO}_2\text{NH}_4\text{PO}_4\cdot 2\text{H}_2\text{O}$  was placed in a nickel tray which was loaded into a nickel tube reactor surrounded by an electrically heated tube furnace. The furnace was then turned on and the reaction zone was heated to a temperature of approximately 450° C. When this temperature was reached, an air flow of 1½ liters per minute was passed through the reactor and maintained for four hours throughout which period the temperature was held at 450° C. The air was then turned off, the temperature raised to 500° C., and an anhydrous HF gas flow of 300 cc. per minute was passed through the reaction zone for four hours. The furnace was then turned off, the reaction zone permitted to cool, and the substantially pure  $\text{UO}_2\text{F}_2$  product removed.

Analysis indicated that the intermediate decomposition compound produced in the above example contained 64.5% U, 26.6%  $\text{PO}_4^{3-}$  and 0.09%  $\text{NH}_4^+$ . The theoretical analysis of uranyl hydrogen phosphate is 65.0% U and 26.0%  $\text{PO}_4^{3-}$ . Thus, substantially complete conversion of uranyl ammonium phosphate to uranyl hydrogen phosphate had been accomplished.

Analysis also indicated that the final hydrofluorination product assayed at 77.0% U (1.34%  $\text{U}^{4+}$ ), 12.8%  $\text{F}^-$ , 0.43%  $\text{PO}_4^{3-}$ , and no detachable  $\text{NH}_4^+$ . The theoretical analysis of  $\text{UO}_2\text{F}_2$  is 77.3% U and 12.3%  $\text{F}^-$ . Thus, the final product was approximately 98%  $\text{UO}_2\text{F}_2$ .

In general, it may be said that the above example is merely illustrative and should not be construed as limiting the scope of our invention which should be understood to be limited only as indicated by the appended claims.

What is claimed is:

1. A method of converting uranyl ammonium phosphate to uranyl fluoride which comprises heating the uranyl ammonium phosphate at a temperature of 300-500° C. until substantially all the uranyl ammonium phosphate is converted to uranyl hydrogen phosphate and contacting said uranyl hydrogen phosphate with anhydrous HF gas at a temperature of 350 to 600° C. until said uranyl hydrogen phosphate is substantially completely converted to  $\text{UO}_2\text{F}_2$ .

2. A method of converting  $\text{UO}_2\text{NH}_4\text{PO}_4\cdot 4\text{H}_2\text{O}$  to  $\text{UO}_2\text{F}_2$  which comprises drying the  $\text{UO}_2\text{NH}_4\text{PO}_4\cdot 4\text{H}_2\text{O}$  at a temperature of approximately 60° C. until said  $\text{UO}_2\text{NH}_4\text{PO}_4\cdot 4\text{H}_2\text{O}$  is substantially all dehydrated to  $\text{UO}_2\text{NH}_4\text{PO}_4\cdot 2\text{H}_2\text{O}$ , heating said  $\text{UO}_2\text{NH}_4\text{PO}_4\cdot 2\text{H}_2\text{O}$  at a temperature of 300-500° C. until substantially all the

$\text{UO}_2\text{NH}_4\text{PO}_4\cdot 2\text{H}_2\text{O}$  is decomposed to uranyl hydrogen phosphate and contacting said uranyl hydrogen phosphate with anhydrous HF gas at a temperature of 350-600° C. until said uranyl hydrogen phosphate is substantially all converted to  $\text{UO}_2\text{F}_2$ .

3. A method of converting  $\text{UO}_2\text{NH}_4\text{PO}_4\cdot 2\text{H}_2\text{O}$  to uranyl fluoride which comprises heating the



10 at a temperature of 300-500° C. until substantially all the  $\text{UC}_2\text{NH}_4\text{PO}_4\cdot 2\text{H}_2\text{O}$  is converted to uranyl hydrogen phosphate and contacting said uranyl hydrogen phosphate with anhydrous HF gas at a temperature of 350 to 600° C. until said uranyl hydrogen phosphate is substantially completely converted to  $\text{UO}_2\text{F}_2$ .

15 4. A method of forming substantially pure uranyl hydrogen phosphate from uranyl ammonium phosphate which comprises heating the uranyl ammonium phosphate at a temperature of 300-500° C. until the decomposition of said uranyl ammonium phosphate to uranyl hydrogen phosphate is substantially complete.

20 5. A method of converting  $\text{UO}_2\text{NH}_4\text{PO}_4\cdot 4\text{H}_2\text{O}$  to uranyl hydrogen phosphate which comprises drying the  $\text{UO}_2\text{NH}_4\text{PO}_4\cdot 4\text{H}_2\text{O}$  at a temperature of approximately 60° C. until said  $\text{UO}_2\text{NH}_4\text{PO}_4\cdot 4\text{H}_2\text{O}$  is substantially all dehydrated to  $\text{UO}_2\text{NH}_4\text{PO}_4\cdot 2\text{H}_2\text{O}$  and heating said



25 at a temperature of 300-500° C. until substantially all the  $\text{UO}_2\text{NH}_4\text{PO}_4\cdot 2\text{H}_2\text{O}$  is decomposed to uranyl hydrogen phosphate.

30 6. A method of forming substantially pure uranyl hydrogen phosphate from  $\text{UO}_2\text{NH}_4\text{PO}_4\cdot 2\text{H}_2\text{O}$  which comprises heating said  $\text{UO}_2\text{NH}_4\text{PO}_4\cdot 2\text{H}_2\text{O}$  at a temperature of 300-500° C. until the resulting decomposition to uranyl hydrogen phosphate is substantially complete.

35 7. A method of converting uranyl hydrogen phosphate to substantially pure  $\text{UO}_2\text{F}_2$  which comprises contacting said uranyl hydrogen phosphate with anhydrous HF gas at a temperature of 350-600° C. until said conversion is substantially complete.

40 8. A method of forming substantially pure



45 from  $\text{UO}_2\text{NH}_4\text{PO}_4\cdot 4\text{H}_2\text{O}$  which comprises heating the  $\text{UO}_2\text{NH}_4\text{PO}_4\cdot 4\text{H}_2\text{O}$  at a temperature of approximately 60° C. and in contact with the ambient atmosphere until said  $\text{UO}_2\text{NH}_4\text{PO}_4\cdot 4\text{H}_2\text{O}$  is dehydrated to



50 9. A process for converting  $\text{UO}_2\text{NH}_4\text{PO}_4\cdot 2\text{H}_2\text{O}$  to substantially pure  $\text{UO}_2\text{F}_2$  which comprises heating said  $\text{UO}_2\text{NH}_4\text{PO}_4\cdot 2\text{H}_2\text{O}$  at a temperature of approximately 450° C. for 2-5 hours, and contacting the resulting uranyl hydrogen phosphate with anhydrous HF gas at a temperature of 350-600° C. for 2-4 hours.

55 10. A method of forming substantially pure



60 from  $\text{UO}_2\text{NH}_4\text{PO}_4\cdot 4\text{H}_2\text{O}$  which comprises heating the  $\text{UO}_2\text{NH}_4\text{PO}_4\cdot 4\text{H}_2\text{O}$  at a temperature of 50° C.-80° C. and in contact with the ambient atmosphere until said  $\text{UO}_2\text{NH}_4\text{PO}_4\cdot 4\text{H}_2\text{O}$  is dehydrated to  $\text{UO}_2\text{NH}_4\text{PO}_4\cdot 2\text{H}_2\text{O}$ .

65 **References Cited in the file of this patent**

Sutton: Chemical News, volume 1, pages 97-8 (1860).

Kitchin: Chemical News, volume 27, page 199 (1873).

Friend: Textbook of Inorganic Chemistry, volume 7, part 3, page 330 (1926). Published by Charles Griffin and Company, London.

UNITED STATES PATENT OFFICE  
CERTIFICATE OF CORRECTION

Patent No. 2,795,479

June 11, 1957

Seymour Bernstein et al.

It is hereby certified that error appears in the printed specification of the above numbered patent requiring correction and that the said Letters Patent should read as corrected below.

Column 3, line 52, for "detachable NH<sub>4</sub>" read --detectable NH<sub>4</sub>+-; column 4, line 60, for "4HO<sub>2</sub>" read --4H<sub>2</sub>O--.

Signed and sealed this 24th day of September 1957.

(SEAL)

Attest:

KARL H. AXLINE

Attesting Officer

ROBERT C. WATSON  
Commissioner of Patents